

## UNITED STATES PATENT OFFICE

2,256,553

## TIRE CORD

Camille Dreyfus, New York, N. Y.

No Drawing. Application June 15, 1939,  
Serial No. 279,259

5 Claims. (Cl. 57—140)

This invention relates to the treatment of textile yarns, filaments and the like made of cellulosic materials, particularly those made of or containing regenerated cellulose, partially saponified cellulose esters, or cotton, in order to improve their properties.

An object of this invention is the treatment of cellulosic yarns or filaments in order to improve their wearing qualities.

Another object of this invention is the treatment of yarns or filaments made of or containing cellulosic material so as to render them more suitable for use in the manufacture of tire cords.

A further object of this invention is to maintain as much as possible the strength of yarns or filaments made of or containing cellulosic material during the manufacture of tire cords. Other objects of the invention will appear from the following detailed description.

In the manufacture of tires and other operations wherein yarns are exposed to relatively high temperatures and/or atmospheres of relatively low humidity, yarns of cellulosic material tend to lose part of their strength particularly when subjected to torsional stresses. I have found that this is partly due to the loss by the yarns of natural moisture under such conditions.

I have found that if yarns made of cellulosic materials are treated with hygroscopic liquid that has no deleterious effect on the yarns, because the yarns are protected against the loss of all moisture, the yarns do not suffer appreciable loss of strength when exposed to relatively high temperatures and/or relatively dry atmosphere. As a result, cord formation is facilitated and the resulting tires have increased strength and wearing properties.

While this invention is of value in connection with the treatment of yarns, threads or cords made of filaments of fibers of cellulosic material, such as partially or completely saponified cellulose acetate or other cellulose esters, or other regenerated cellulose such as from viscose or cuprammonium solutions of cellulose, cotton, flax, etc., particularly good results are obtained in connection with the treatment of yarn of high tenacity obtained by the saponification of cellulose acetate or other cellulose ester yarn that has been stretched before saponification, while softened, up to 200 to 500%.

The cellulosic yarn may be treated with any relatively non-volatile hygroscopic liquid, provided it has no deleterious effect either at ordinary temperatures or the higher temperatures, such as 125 to 150° C. prevailing during vulcani-

zation, to which they are exposed during treatment or use. Generally as hygroscopic material we prefer to employ relatively non-volatile polyhydric alcohols or their partial ethers or esters, such as glycerol, ethylene glycol, propylene glycol, diethylene glycol, the monoethyl ether of diethylene glycol, monoacetyl (glyceryl monoacetate).

In order to stabilize the solution in which the hygroscopic liquid is applied against change of volume, viscosity or concentration due to evaporation or absorption of water, it is preferable to add a quantity of water substantially equal to the amount of water these liquids tend to absorb from the air, the amount of water being 30% in the case of diethylene glycol, 13% in the case of ethylene glycol and 33% in the case of glycerol.

If desired, the hygroscopic material may be applied in conjunction or separately with other materials such as lubricants containing tricresyl phosphate, sulfonated vegetable oils, and/or soaps.

The hygroscopic material may be applied to the yarns before, during or after any textile operation to which they are subjected. Thus it may be applied to the yarns or filaments during any winding or twisting operation by passing the same in contact with a wick, roller, disc or other furnishing device that dips into the liquid comprising the hygroscopic material. The yarns or filaments may be drawn through a solution or emulsion of the hygroscopic material or the same may be sprayed upon the yarn. The hygroscopic material may also be applied to the yarns or filaments in hank form by hand dipping methods, or the yarns may be treated with the hygroscopic material by padding or spraying after they have been formed into a cord.

The amount of hygroscopic material applied will vary with the type of yarn and especially with the type of cord into which it is to be converted. Thus heavy duty cords such as are used in the manufacture of truck tires will require a higher proportion of hygroscopic material than will cords which are to be used in a tire for a passenger automobile. We have found that excellent results are obtained where 1 to 10.0% of hygroscopic material on the weight of the yarn is applied to and/or retained by the yarn.

50 The following is an example of an application of the invention, it being understood that this is given by way of illustration only.

*Example*

Travelling yarns of regenerated cellulose of about 270 denier obtained by the saponification

of a cellulose acetate yarn whose filaments had been stretched 200% before saponification, having a twist of about 5 turns per inch, are contacted with a wick which dips into a bath consisting of 75% of glycerine and 25% of water. The wick is adjusted so that 5% of the glycerine, on the basis of the weight of the yarn, is retained by the travelling yarn. The yarn is thus uniformly and evenly impregnated with the glycerine.

Yarns thus treated are plied by twisting four ends together 14 turns per inch, left. Three plies thus formed are then twisted about 12 turns per inch, right, in order to obtain a cable suitable for cords in tire manufacture. The travelling yarn after it receives the lubricant may pass directly to the plying and cabling machines.

The treated yarns when incorporated in a tire maintains markedly improved strength as compared with similar yarns untreated.

It is to be understood that the foregoing detailed description is merely given by way of illustration and that many variations may be made therein without departing from the spirit of my invention.

Having described my invention, what I desire to secure by Letters Patent is:

1. Tire cords of improved strength comprising cellulosic yarns having a hygroscopic liquid incorporated therein.
- 5 2. Tire cords of improved strength comprising cellulosic yarns having incorporated therein a hygroscopic liquid selected from the group consisting of polyhydric alcohols, their partial ethers and partial esters.
- 10 3. Tire cords of improved strength comprising regenerated cellulosic yarns having incorporated therein a hygroscopic liquid selected from the group consisting of polyhydric alcohols, their partial ethers and partial esters.
- 15 4. Tire cords of improved strength comprising regenerated cellulose yarns obtained by the saponification of highly stretched cellulose acetate yarns, said regenerated cellulose yarns having incorporated therein a hygroscopic liquid selected from the group consisting of polyhydric alcohols, their partial ethers and partial esters.
- 20 5. Tire cords of improved strength comprising regenerated cellulose yarns obtained by the saponification of highly stretched cellulose acetate yarns, said regenerated cellulose yarns having glycerine incorporated therein.

CAMILLE DREYFUS.